

Nov. 10, 1936.

W. SINGLETON ET AL

2,060,534

LEAD ALLOY

Filed July 25, 1935

Fig. 1.



Fig. 2.



Fig. 3.

15



William Singleton, Wm. Hulme  
& Brinsley Jones  
By Watson, Coit, Moore & Grundy  
ATTYS.

## UNITED STATES PATENT OFFICE

2,060,534

## LEAD ALLOY

William Singleton, Wembley, William Hulme, Bush Hill Park, and Brinley Jones, Ealing, London, England, assignors to Goodlass Wall and Lead Industries Limited, London, England, a British company

Application July 25, 1935, Serial No. 33,180  
In Great Britain November 19, 1931

26 Claims. (Cl. 148—33)

This invention relates to improvements in lead and lead alloys and to processes of manufacturing and treating the same, and has for its principal object the provision of a lead or alloy of lead or articles containing the same with improved mechanical properties and greater resistance to corrosive influences. This application is a continuation in part of our prior application for Letters Patent Serial No. 641,320, filed November 10, 4th, 1932.

It is known that lead can be alloyed with tellurium, but such alloys have not, so far as we are aware, received commercial application prior to the development of the present invention. We have now discovered that lead to which a very small proportion of tellurium has been added has entirely new properties, even though in such alloys the proportion of tellurium may be so small that the material may almost be regarded as lead rather than as an alloy of lead with tellurium, but for convenience in this specification the metal is referred to as a lead tellurium alloy. It has also been found that advantages are realized by the addition of tellurium to conventional alloys of lead with other metals, for instance with antimony, tin and cadmium, or alloys of lead with various combinations of these other metals, such alloys as well as the lead tellurium alloy being referred to broadly herein as lead-base alloys.

One very material advantage resulting from the addition of tellurium to lead even when the proportion of tellurium added is very small, for example of the order of 0.02% of tellurium, resides in the fact that although the material as cast is almost as soft as ordinary pure commercial lead it is nevertheless capable of being permanently work-hardened or toughened so that it has a much increased tensile strength of over 50% after rolling, the bulk of the increased strength being permanently retained at ordinary temperatures. The tensile strength of commercial lead is approximately doubled when tellurium of the order of 0.06% is added. It is also found that lead tellurium alloys within the scope of this invention are in general more resistant to corrosion by chemically active materials such as concentrated acids, for instance sulphuric and phosphoric acid, than is ordinary lead. Lead which is improved by the addition of tellurium in accordance with the present invention is less readily attacked by boiling sulphuric acid and even extremely small proportions of tellurium, such for example as 0.04% to 0.07% of tellurium, serve to raise the so-called "flash point" of lead

when subjected to sulphuric acid, temperatures of 310° C. or over being necessary to reach the "flash point", while in proportions of about 0.07% or over the tellurium imparts to the lead such resistance to attack that it will not "flash" even when exposed to boiling sulphuric acid.

In general in the practice of our invention we prefer to use quantities of tellurium ranging from not substantially below 0.02%, to not substantially above 0.1%. Quantities of tellurium materially in excess of the latter figure have been found to develop in lead or lead alloy adverse characteristics unless special precautions are observed in the preparation of the material. Quantities substantially below that of 0.02% are insufficient for the development of appreciable improvement from a practical standpoint.

Thus one of the principal difficulties encountered when the percentage of tellurium is materially greater than 0.1% is the tendency of the tellurium to segregate when using the ordinary method of casting. It is found, for instance, that when the proportion of tellurium added to lead or a lead alloy does not exceed 0.1%, the tellurium is distributed substantially uniformly throughout a cast billet. On the other hand, if the quantity of tellurium be increased to 0.12%, the billet is found to contain considerably more tellurium in the upper than in the lower portions, and this lack of uniform distribution persists when the billet is subsequently rolled out or extruded into a relatively thin section. If a quantity of tellurium as great as 0.14% is introduced, the irregularity of distribution of the tellurium in the cast billet is quite pronounced, approaching rather closely that observed when much larger quantities are used, say up to 0.24%; in other words, there is a rather sharp break in the curve representing the tendency of tellurium to segregate with a small increase in the quantity of tellurium over 0.1%, and this lack of uniformity is most undesirable.

It can be demonstrated that quantities of tellurium and lead in the neighbourhood of 0.05% to 0.06% represent approximately the solid solubility of tellurium in lead, but it is important to note that larger quantities of tellurium up to 0.1% can be introduced without inducing material segregation with the ordinary method of casting. In fact, we have found in general that the optimum quantity of tellurium as regards resistance to corrosion combined with improved mechanical characteristics is about 0.07%, and a preferred range for the practice of our invention lies between 0.06% and 0.1%.

One of the most important improvements in lead or lead alloys obtained by the addition of tellurium thereto in the indicated proportions is the increased strength, toughness and hardness resulting from cold working of the improved material. Thus while lead containing a small proportion of tellurium is quite ductile in the soft condition and may be bent or fashioned as readily as pure commercial lead, it exhibits the extremely important property of work hardening when subjected to cold working and even in the fully cold-worked condition the ductility of the alloy is such that it can be bent double without fracture. For instance, soft commercial pure lead has a tensile strength of the order of 2,100 lbs. per square inch, and a hardness in the rolled sheet of between four and five on the Brinell scale. An alloy of similar lead to which 0.02% of tellurium had been added, was found after cold rolling to have a tensile strength of 3,875 lbs. per square inch, and a hardness of seven to eight on the Brinell scale while the addition of 0.04% tellurium to the same lead, gave a product having a tensile strength of 5,000 lbs. per square inch. Higher tensile strengths have been observed after cold rolling when larger quantities of tellurium up to 0.1% were added to lead. The increased tensile strength is accompanied by toughness and the worked alloy is ductile up to the limit of 0.1%.

Lead tellurium alloy when extruded or worked at elevated temperatures is soft and varying degrees of toughness may be obtained by varying the temperature of extrusion or working. It has been observed that when samples of hot-extruded lead tellurium alloy and commercial lead are tested in a tensile strength testing machine there is marked difference in the behaviour of these two materials. In the case of the former material the uniform distribution of strain as a result of work-hardening is such that the material elongates more regularly and to a considerably greater degree than the commercial lead before fracture takes place. For example when test pieces of the two materials of the same size were tested to breaking point in the same tensile strength testing machine at a rate of elongation of  $\frac{1}{2}$  of an inch per minute the lead tellurium alloy showed an increase of 100% in elongation over that of commercial lead, measured over a gauge length of 8 inches. In spite of the reduction of cross section due to this elongation the breaking load of the tellurium lead test piece, before fracture, exceeded that of the pure lead.

The results of cold work, e. g. higher tensile strength and toughening, would appear in large measure to be retained indefinitely at normal atmospheric temperatures; at elevated temperatures annealing takes place.

If the strength and toughness of the tellurium lead alloy is not fully developed by cold working prior to or in the fashioning of the completed article from which it is formed, the article thus produced is capable of developing additional toughness and strength if subjected to strain or deformation when in use, and this is particularly important where it is desired to produce an article having the maximum softness and ductility with latent power to develop when necessary a materially increased resistance to mechanical strain.

Thus manufactured articles such as pipes or cable sheathing which are formed of this alloy, for example, by hot extrusion, although soft in

their first manufactured state, and easy to work, toughen when subjected to cold work. Consequently, pipes under pressure, if they should yield in any given place, automatically strengthen themselves at that point, resulting in more even expansion of the pipe. Thus, for example pipes of the alloy have been found to withstand twice the number of freezings before bursting than can be withstood by pipes of ordinary commercial lead treated similarly and at the same time. It is a remarkable property of the alloy that in the soft, i. e. unworked state it has a fatigue resistance nearly three times as great as that of ordinary commercial lead. Long applied stresses resulting from expansion and contraction, such as are obtained during variation of temperature, cause not only continued deformation of ordinary lead but ultimately fracture. Lead tellurium alloy can withstand such stresses more satisfactorily since the tendency to flow is automatically checked by the work-toughening of the material. Sheet made from lead tellurium alloy is less liable to thermal creep.

Microscopic examination shows that alloys according to this invention are less susceptible to grain growth, due to heat treatment, than ordinary commercial lead. Due to the fine grain of extruded tellurium lead these products have a very smooth surface and are superior in appearance to ordinary commercial lead.

In ordinary lead, when deformed under stress, the degree of uniformity of the distribution of deformation depends to a large extent on the uniformity and size of the grains. Uniformity of grain size is not so important where grain size is small since defined grain itself ensures more uniform distribution of deformation, but with large areas of very large grains with adjoining areas of extremely small grains (coarse-grained metal) such as generally occurs in ordinary commercial lead, stresses are not uniformly distributed and therefore the deformation is not uniform.

The addition of tellurium to lead raises the temperature of recrystallization and produces changes in the crystalline structure of the lead which, by making it more difficult for the grains to change their direction of orientation, restrains grain growth and so reduces considerably the liability to intercrystalline cracking. The alloy therefore if given initially fine grain retains it and so responds to stress in a more uniform manner than ordinary lead.

The practical effects which result from the foregoing are clearly illustrated in the comparative behaviour of ordinary commercial lead and tellurium lead, when subjected to strain. In the case of ordinary commercial lead, where the structure is generally irregular, strains are unevenly distributed and localized concentration causes recrystallization so that favourable conditions for intercrystalline cracking are established. In the case of tellurium lead in which there is a refined and uniform structure, strain is much more evenly distributed so that the concentration of strain, which occurs in ordinary commercial lead, is absent in tellurium lead and the possibility of intercrystalline cracking very markedly reduced.

No difficulty has in the past been experienced in increasing the strength of lead as measured by the effort required to bend or work metal manually, to increase the Brinell hardness, or raise the fatigue limit and alloys of lead with antimony, tin and cadmium and various com-

binations of the latter have been employed for these purposes for many years. Increased strength in such cases has only been obtained by sacrificing softness, ductility, and other inherent 5 and valuable properties which are characteristic of soft lead. It is found, however, that in accordance with the present invention, the characteristics of these alloys of lead with other metals can be substantially improved by the use 10 of small quantities of tellurium of the order hereinbefore mentioned. Thus the present invention contemplates the addition of tellurium to alloys of lead containing antimony not in excess of 20%, tin not in excess of 70%, or cadmium not 15 in excess of 15%, or to ternary alloys such as lead-antimony-cadmium and lead-tin-cadmium, and to quaternary alloys containing all of these elements in which the proportion of any one of the elements does not exceed that indicated. 20 The addition of tellurium is found particularly valuable in lead-base alloys containing a major proportion of lead and particularly in those alloys of lead with antimony, cadmium, and/or tin which are commonly employed in pipe or cable 25 sheathing and in which lead is present in amount not less than 85% or 90%.

The following examples are given as illustrative of lead-base alloys lying within the indicated field which exhibit markedly superior characteristics upon the addition of quantities of tellurium 30 not substantially greater than 0.1%.

#### Example I

|                 | Per cent |
|-----------------|----------|
| 35 Antimony     | 1        |
| Tellurium       | 0.06     |
| Commercial lead | Balance  |

This alloy showed a strength in the cold rolled condition of 5,700 lbs. per square inch with an 40 elongation on an eight inch length of 12½%. When tellurium was omitted the tensile strength was only 4,550 lbs. per square inch and the elongation 20%. Figure 1 shows a stress-strain diagram for the alloy compared with a similar 45 alloy not containing tellurium and this diagram is given as a typical example of the effect of tellurium additions both on plain lead and lead containing other metals such as antimony.

The effect of annealing for half an hour at 50 200° C. was to cause recrystallization and softening with the result that the alloy containing tellurium had a tensile strength of 3,500 lbs. per square inch and an elongation of 45%, whereas 55 when tellurium was omitted the tensile strength of the sample similarly treated was only 3,080 lbs. per square inch and the elongation 41%. The corresponding stress-strain diagram is shown in Figure 2.

This alloy is suitable for use in extrusion 60 processes owing to the stability imparted by the tellurium to the grain structure at elevated temperatures such as are used in extrusion. The effect of annealing the antimonial lead containing tellurium for half an hour at 200° C. or of 65 high temperature treatment such as extrusion is to produce a fine grain upon recrystallization, whereas similar annealing when tellurium is absent produces a very coarse grain upon recrystallization, the grain size being quite ten times as 70 great in linear dimensions when the tellurium is omitted.

Antimony lead alloys are particularly susceptible to "hot shortness" and give serious difficulties during extrusion. The addition of tellurium 75 by producing a fine and stable structure, reduces

the liability to "hot shortness", and permits a wider range of extrusion conditions.

#### Example II

|                 | Per cent |
|-----------------|----------|
| Antimony        | 8        |
| Tellurium       | 0.07     |
| Commercial lead | Balance  |

This example shows the application of the invention to a high antimony alloy such as is frequently used for its resistance to chromic acid solutions. This alloy, when tested in a chromium-plating bath as used in industry showed a loss of weight per 100 square centimetres per twenty-four hours of 0.22 gram. When the tellurium 15 was omitted the loss of weight was 19.1 grams for the same time and area. This illustrates in a striking way the superior corrosion resistance of the alloy containing tellurium.

#### Example III

The following is an example of a cadmium lead alloy containing tellurium:

|                 | Per cent |
|-----------------|----------|
| Cadmium         | 0.5      |
| Tellurium       | 0.07     |
| Commercial lead | Balance  |

The addition of tellurium to this cadmium alloy had a marked effect in increasing the tensile strength and elongation of both cold-rolled and annealed materials.

After cold-rolling the strength of the alloy containing tellurium was 4,080 lbs. per square inch, against 3,500 lbs. per square inch when tellurium was omitted and the elongation was 32.5% 35 against 30%. After annealing for half an hour at 200° C. the tensile strength was 3,820 lbs. per square inch and elongation 45% against a strength of 3,500 lbs. per square inch and elongation of 34% when tellurium was omitted. Comparison of the figures of the tellurium-lead-cadmium alloy in the rolled and annealed condition shows that the rolling increased the tensile strength and reduced the elongation, thus 40 indicating work hardening, which was substantially absent when tellurium was omitted from the alloy. As in the case of the other alloys herein dealt with the tellurium has the effect of stabilizing the grain structure at elevated temperatures and preventing grain growth through 45 annealing.

#### Example IV

The following is an example of a tin alloy.

|                 | Per cent |
|-----------------|----------|
| Tin             | 3        |
| Tellurium       | 0.07     |
| Commercial lead | Balance  |

This alloy showed marked increase of strength 60 and in addition showed work hardening properties as compared with an alloy from which tellurium was omitted. The tensile strength after rolling was 5,200 lbs. per square inch and elongation, measured on a length of eight inches, 12%, 65 whereas a 3% tin-lead alloy without tellurium had a tensile strength of 3,760 lbs. per square inch after rolling with an elongation of 45%.

After annealing for half an hour at 200° C. the alloy-containing tellurium showed a tensile 70 strength of 3,930 lbs. per square inch and an elongation of 49%; while the tin lead alloy without tellurium similarly annealed showed a strength of 3,520 lbs. per square inch and elongation of 38%.

Resistance to grain growth upon annealing similar to that shown in the previously mentioned alloys was revealed in this case. In other words the alloy is more stable under heat treatment and this enables it to be better extruded and permits a larger range of extrusion conditions than is possible with the alloy free from tellurium.

*Example V*

|                 | Per cent |
|-----------------|----------|
| Tin             | 30       |
| Tellurium       | 0.06     |
| Commercial lead | Balance  |

*Example VI*

|                 | Per cent |
|-----------------|----------|
| Tin             | 50       |
| Tellurium       | 0.06     |
| Commercial lead | Balance  |

20 The alloys of Examples V and VI are solders, Example V being a plumber's solder and Example VI a tinman's solder. They are characterized by a greater fluidity near the solidifying point than ordinary solder and are therefore easier to work.

25 The tinman's solder runs particularly well under the iron.

*Example VII*

The following is an example of a type of bearing metal.

|                 | Per cent |
|-----------------|----------|
| Tin             | 10       |
| Antimony        | 15       |
| Tellurium       | 0.06     |
| Commercial lead | Balance  |

35 The resistance to recrystallization and to coarsening of grain under heat which is imparted by tellurium is a distinct benefit in metals of this class.

40 It is found that the addition of tellurium in the foregoing alloys not only renders these alloys susceptible to toughening by cold working and therefore produces in them the characteristic properties of the binary lead tellurium alloy, but

45 the known desirable properties of these alloys are retained. Due to the greater stability of structure imparted to these alloys by the addition of tellurium the invention renders available a more extensive range of extrusion temperatures than hitherto, and in general the alloys are improved 50 in the same manner as is commercial lead when tellurium is introduced.

A further important advantage of the invention lies in the fact that the hardness, strength, 55 or toughness of manufactured lead articles can be controlled. Hard or tough articles can be manufactured by cold working the metal, and articles of degrees of toughness or hardness varying over a wide range can be obtained at will 60 by working at regulated temperatures or variation of extent of working or by cold working with annealing.

65 The following example is illustrative of the manner in which the characteristics of the material may be controlled:—

*Example VIII*

Certain effects of work hardening upon the physical characteristics of the tellurium-containing alloys of lead and of lead with other metals 70 have already been pointed out in the examples given hereinabove. The following relates to an alloy consisting almost entirely of lead, but containing tellurium to the extent of 0.06%. This 75 was rolled from cast ingots six inches thick into

the form of sheet about one-eighth of an inch thick and tests were made in comparison with similar lead containing no tellurium. Another ingot of the same materials was extruded into strip-form for purposes of comparison. The following table gives the results:—

|                                                   | Commercial lead | Commercial lead containing tellurium | Elongation under rapid rate of straining (2" per min.) | 10 |
|---------------------------------------------------|-----------------|--------------------------------------|--------------------------------------------------------|----|
|                                                   |                 |                                      |                                                        |    |
| (a) 7 days after rolling                          | 2,200           | 4,000                                | Per cent 15                                            |    |
| (b) As (a) but after annealing 3 hours at 100° C. | 2,300           | 3,240                                | 37                                                     |    |
| (c) As (a) but after annealing 7 days at 100° C.  | 2,300           | 3,135                                | 33                                                     |    |
| (d) As (a) but after annealing 3 hours at 150° C. | 2,300           | 3,230                                | 35                                                     | 20 |
| (e) As (a) but after annealing 7 days at 150° C.  | 2,300           | 2,940                                | 34                                                     |    |
| (f) As (a) but after annealing 3 hours at 200° C. | 2,300           | 2,880                                | 35                                                     |    |
| (g) As extruded                                   | 2,300           | 2,700                                | 55                                                     |    |

25 While as has been hereinbefore indicated, for many purposes the critical upper limit of tellurium is not substantially above 0.1%, as established by the development of certain adverse characteristics of which the most important is the segregation of the tellurium, we may under some 30 circumstances practice our invention by the employment of still greater quantities of tellurium, for instance proportions up to about .25%. While in the absence of special conditions of preparation these increased quantities of tellurium render the material much less satisfactory, it is nevertheless possible to apply to such alloys the regulatory steps herein suggested whereby substantially the desired degree of toughness or hardness can be obtained and for some purposes the tendency 40 of the tellurium to segregate does not constitute a serious disadvantage.

45 Reference is made herein to special conditions of manufacture which may be observed in the formation of the alloy or the article of which the 50 alloy is composed and which have been found to reduce to a material extent the tendency of the tellurium to segregate when employed in quantities materially greater than 0.1%. One such 55 method of procedure is to cast the molten metal in the form of thin plates, and to immediately chill the cast metal. It is found that with this process substantial uniformity of distribution of the tellurium can be secured and an improvement 60 of the resulting alloy, similar to that described hereinbefore when smaller quantities of tellurium are used, can be obtained even though quantities of tellurium as high as 2% are added. This procedure is of course applicable not only to the 65 treatment of lead but to the treatment of alloys of lead with tin, cadmium, and antimony as hereinbefore described.

The following example is illustrative of this method as applied to the formation of battery plates, in which field it is particularly suitable 70 owing to the conventional employment of lead in the form of thin plates:—

*Example IX*

A Planté type cast battery plate was produced 70 as shown in the accompanying drawing, Figure 3. In the drawing 11 represents the working part of the plate which contained nine sections of grooved structure intersected by ribs 12. The plate had a lug 13 for terminal connections, a supporting lug 75

- 14 and was cast with a scrap section 15 along the side which lay uppermost in the mould. An iron mould was used so that the casting was chilled during setting.
- 5 The dimensions were as follows:—
- Length (horizontally in the drawing) 18 centimetres  
 Width (of active portion of plate) 13 centimetres  
 10 Width (of scrap section) 4 centimetres  
 Dimensions of terminal lug:  
 Length 4 centimetres  
 Width 2 centimetres  
 Overall thickness of plate 9 millimetres
- 15 On the drawing the percentages of tellurium which were separately determined in each section of the plate are clearly marked and it will be observed that they show a substantial uniformity throughout the plate. This uniformity is due to 20 the conditions of casting in a thin section rapidly chilled. Otherwise marked segregation of the tellurium would have occurred.
- It will be understood that the word "lead" as used herein is intended to cover either chemically 25 pure lead, or electrolytic lead, or lead in the usual commercial form in which small quantities of other metals, e. g. copper, nickel and bismuth are sometimes present. It will also be appreciated that in the appended claims it is desired to cover 30 alloys such as those described in which impurities may be present in the completed alloy as well as in any of the components thereof and alloys corresponding to those described but containing ingredients which are inert or which do not contribute to the production of a result differing in any material degree from that contemplated by the present applicants.
- We claim:—
1. A lead-base alloy consisting substantially of 40 lead and containing a small proportion of tellurium in amount of from about 0.02% to about 0.1% of the whole alloy, said alloy being characterized by increased corrosion resistance and strength and amenability to hardening by cold working as compared with similar lead-base alloys free from tellurium.
2. A lead-base alloy consisting substantially of lead, containing antimony in relatively small and beneficial amount, and containing a small proportion of tellurium in amount of from about 0.02% to about 0.1% of the whole alloy, said alloy being characterized by increased corrosion resistance and strength and amenability to hardening by cold working as compared with similar lead-base alloys free from tellurium.
3. A lead-base alloy consisting substantially of lead, containing tin in relatively small and beneficial amount, and containing a small proportion of tellurium in amount of from about 0.02% to about 0.1% of the whole alloy, said alloy being characterized by increased corrosion resistance and strength and amenability to hardening by cold working as compared with similar lead-base alloys free from tellurium.
4. A lead alloy composed entirely of lead and a small proportion of tellurium in amount of from about 0.02% to about 0.1% of the whole alloy, said alloy being characterized by increased corrosion resistance and strength and amenability to hardening by cold working as compared with similar lead-base alloys free from tellurium.
- 5 An extruded elongated tubular article formed of the lead-base alloy described in claim 1.
6. Pipe formed of the lead-base alloy described 75 in claim 1.
7. Cable sheathing formed of the lead-base alloy described in claim 1.
8. Extruded articles formed of the lead-base alloy described in claim 1.
9. A lead-base alloy consisting substantially of lead, containing antimony in amount not exceeding 20%, and containing a small proportion of tellurium in amount of from about 0.02% to about 0.1% of the whole alloy, said alloy being characterized by increased corrosion resistance and strength and amenability to hardening by cold working as compared with similar lead-base alloys free from tellurium. 5
10. A lead-base alloy consisting of at least 85% lead, any remainder being composed of at least one metal selected from the group consisting of tin, antimony and cadmium, and a small proportion of tellurium in amount of from about 0.02% to about 0.1%, said tellurium being distributed substantially uniformly throughout said 20 alloy, said alloy being characterized, as compared with alloys otherwise similar but containing no tellurium, by substantially smaller grain size and by increased resistance to grain growth and inter-crystalline cracking. 25
11. An elongated tubular article formed of a lead-base alloy consisting of at least 85% lead, any remainder being composed of at least one metal selected from the group consisting of tin, antimony and cadmium, and a small proportion 30 of tellurium in amount not exceeding 0.1% and not less than about 0.02%.
12. Pipe formed of a lead-base alloy consisting of at least 85% lead, any remainder being composed of at least one metal selected from the group consisting of tin, antimony and cadmium, and a small proportion of tellurium in amount not exceeding 0.1% and not less than about 0.02%. 35
13. Cable sheathing formed of a lead-base alloy consisting of at least 85% lead, any remainder being composed of at least one metal selected from the group consisting of tin, antimony and cadmium, and a small proportion of tellurium in amount not exceeding 0.1% and not less than about 0.02%. 40
14. An extruded elongated article formed of a lead-base alloy consisting of at least 85% lead, any remainder being composed of at least one metal selected from the group consisting of tin, antimony and cadmium, and a small proportion 50 of tellurium in amount not exceeding 0.1% and not less than about 0.02%.
15. A lead-base alloy consisting substantially of lead and containing a small proportion of tellurium in amount of from about 0.06% to about 0.1% of the whole alloy, said alloy being characterized by increased corrosion resistance and strength and amenability to hardening by cold working as compared with similar lead-base alloys free from tellurium. 55
16. A lead alloy composed entirely of lead and a small proportion of tellurium in amount of from about 0.06% to about 0.1% of the whole alloy, said alloy being characterized by increased corrosion resistance and strength and amenability to hardening by cold working as compared with similar lead-base alloys free from tellurium. 60
17. A lead-base alloy consisting substantially of lead, containing a metal selected from the group consisting of antimony, tin and cadmium, and containing a small proportion of tellurium of the order of from 0.06% to 0.1% of the whole alloy, said alloy being characterized by increased corrosion resistance and strength and amenability to 70
- 75

to hardening by cold working as compared with similar lead-base alloys free from tellurium.

18. Cold-worked material formed of an alloy consisting substantially of lead and containing a small proportion of tellurium in amount of from about 0.02% to about 0.1% of the whole alloy, said alloy being characterized by increased corrosion resistance and strength and amenability to hardening by cold working as compared with similar lead-base alloys free from tellurium.

19. Cold-worked material formed of an alloy consisting substantially of lead and containing a small proportion of tellurium in amount of from about 0.02% to about 0.25% of the whole alloy, said alloy being characterized by increased corrosion resistance and strength and amenability to hardening by cold working as compared with similar lead-base alloys free from tellurium.

20. A lead-base alloy composed entirely of lead and a small proportion of tellurium less than 0.25% but not less than about 0.02%, said alloy having increased toughness and strength imparted thereto by cold working.

21. A lead-base alloy consisting of at least 85% lead, any remainder being composed of at least one metal selected from the group consisting of tin, antimony and cadmium, and a small proportion of tellurium in amount less than 0.25% and not less than about 0.02%, said alloy having increased toughness and strength imparted thereto by cold working.

22. A method of permanently increasing to a controlled extent the degree of toughness and strength of a lead-base alloy consisting substantially of lead and containing a small proportion of tellurium less than 0.25% but not less than about 0.02%, which comprises working the alloy to toughen and strengthen the same while maintaining a temperature sufficient to partially offset the toughening and strengthening effect of working.

23. A method of permanently increasing to a

controlled extent the degree of toughness and strength of a lead-base alloy consisting substantially of lead and containing a small proportion of tellurium less than 0.25% but not less than about 0.02%, which comprises the successive steps of cold working the alloy to toughen and strengthen the same, and heating the alloy sufficiently to partially offset the toughening and strengthening effect of working.

24. A method of permanently increasing to a controlled extent the degree of toughness and strength of a lead-base alloy consisting of at least 85% lead, and remainder being composed of at least one metal selected from the group consisting of tin, antimony and cadmium, and a small proportion of tellurium in amount less than 0.25% and not less than about 0.02%, which comprises working the alloy to toughen and strengthen the same while maintaining a temperature sufficient to partially offset the toughening and strengthening effect of working.

25. A method of permanently increasing to a controlled extent the degree of toughness and strength of a lead-base alloy consisting of at least 85% lead, any remainder being composed of at least one metal selected from the group consisting of tin, antimony and cadmium, and a small proportion of tellurium in amount less than 0.25% and not less than about 0.02%, which comprises cold working the alloy to toughen and strengthen the same, and thereafter heating the alloy sufficiently to partially offset the toughening and strengthening effect of working.

26. A lead-base alloy consisting substantially of lead and containing a small proportion of tellurium in amount of from about 0.02% to about 0.10%, said alloy having increased toughness and strength imparted thereto by cold working.

WILLIAM SINGLETON. 40  
WILLIAM HULME.  
BRINLEY JONES.